

June 7, 1932.

A. MURRAY

1,861,872

PHOTOMECHANICAL REPRODUCTION FROM HALF TONES OR LINE NEGATIVES

Filed March 12, 1930

*Fig. 1.*



*Fig. 2.*



*Fig. 3.*



*Fig. 4.*



*Fig. 5.*



*Fig. 6.*



*Fig. 7.*



*Fig. 8.*



Alexander Murray.

Inventor

By *M. M. Perraud*

Attorney

## UNITED STATES PATENT OFFICE

ALEXANDER MURRAY, OF ROCHESTER, NEW YORK, ASSIGNOR TO EASTMAN KODAK COMPANY, OF ROCHESTER, NEW YORK, A CORPORATION OF NEW YORK

## PHOTOMECHANICAL REPRODUCTION FROM HALF TONES OR LINE NEGATIVES

Application filed March 12, 1930. Serial No. 435,077.

This invention relates to photo-engraving and lithography, and more particularly to photo-mechanical reproductions from half-tone or line negatives.

5 One object of the invention is to provide copies or duplicates of photo-mechanical halftones or line negatives by a cheap and convenient method.

Another object is to provide a convenient 10 and time-saving method of obtaining color proofs before the final printing plate has been made. According to present practice by the usual indirect method used in lithography for obtaining the screen color positive, it is not 15 possible to obtain a proof of any one of the color plates until the final plate has been made. If the retouching is incorrect or for 20 any reason the plate is imperfect, it is necessary either to discard one or two plates and the final lithographic plate, or to make an additional correction plate, thereby adding greatly to the expense of the process. By my 25 invention it is possible to obtain a color proof from the screen positive made from the original color separation negative before making the screen color negative and printing the latter on the final plate. It is then easily possible to correct or retouch so as to give the 30 proper color rendering at an early stage so that the final stages of preparing the screen negative and the lithographic surfaces need not be repeated.

A method is needed for making a negative or positive containing stencil-like dots from 35 a negative or positive containing soft or graded dots. Also it frequently happens that a photo-mechanical negative becomes damaged or broken in use and it will be desirable to have a copy or duplicate of the same. In other cases it would be desirable to 40 have a number of such negatives without the trouble of producing them in the original manner. In still other cases the duplicate could be kept as a matter of record. The 45 present invention represents a very cheap, convenient and rapid method of making such duplicates.

The method I propose is similar in some respects to that proposed for making negatives 50 from printing forms described in my appli-

cation Serial Number 374,238, filed June 27, 1929. The process, however, differs from that disclosed in the former application in several important details.

Reference is made to the accompanying 55 drawing.

Figure 1 is a cross section showing the negative which is to be duplicated and a sensitive layer on to which it is being printed.

Figure 2 shows the sensitive layer after it 60 is inked, developed, and dyed.

Figure 3 shows the sensitive layer after it is inked, developed, dyed and the ink removed.

Figure 4 shows in cross section the process 65 carried out on a plate coated with asphalt.

Figure 5 shows the dye image made from the form shown in Fig. 4.

Figure 6 shows a variation of the method 70 where both an asphalt and shellac layer are used on the support.

Figure 7 shows the asphalt and shellac 75 layer after the portion of the surface consisting of shellac has been removed.

Figure 8 shows the final surface consisting 80 of the dye image and clear shellac.

I will now describe my invention and two 85 of its preferred forms as applied to the making of copies of photomechanical halftones or line negatives or positives, and to the method of making color proofs from them. I do not, of course limit myself to the two forms described.

The invention in its simplest form is applied to the making of duplicates of photomechanical negatives. For this purpose I first prepare a light sensitive surface by coating a sheet of glass or film 1 with a bichromated colloid layer 2 in a manner well known in the art. Examples of the kinds of bichromated colloids which may be used are bichromated albumen, glue or gum arabic. This sensitive coating is, as shown in Fig. 1, placed in contact with the negative to be reproduced and comprising support 3 carrying the image layer 4 and exposed to light under it, rendering insoluble the portions reached by the light. After exposure, the printed surface is uniformly inked with a greasy ink. It is then developed by placing it in water which removes the soluble por- 100

tions not exposed to the light. A very thin residual film 8 of the soluble colloid firmly adheres to the support and this is then flowed with a dye dissolved in a solvent which does not attack the ink, and which forms a continuous film 7 of color on the surface except where the later is protected by the ink. This may or may not penetrate the very thin remaining layer 8 and is shown for purposes of illustration as a separate dye layer 7 in Fig. 2. The film 8 is so thin that it is not readily detectable and its existence is assumed from the fact that dye adheres. At this stage the reproduction consists of a relief colloid design 5 covered with ink 6 and a background of dye 7, as shown in Figure 2. After drying, the ink is removed from the surface of the support by the aid of a solvent, such as benzol, which does not attack the stain or the support. The result (Figure 3) is a negative resembling the original in appearance except that the dark portion consists of dye instead of silver, and consisting of a colloid relief, the thick portions 5 of which are undyed, and the thin portions 8 are dyed.

In developing the colloid surface the temperature of the water to be used will depend on the particular colloid used. In most cases ordinary cold water from the tap will be satisfactory. Other substances may require somewhat warmer water. A stain suitable for use in this process may be made by taking:

|                | Parts |
|----------------|-------|
| Methyl alcohol | 85    |
| Aurine         | 10    |
| Rubine         | 5     |

The above stain is typical of many others which may be used. The dye should be highly soluble and have a strong absorption from 500  $m\mu$  into the near ultra-violet region of the spectrum.

For the purpose of obtaining color proofs from lithographic reproductions, I use a variation of the above method in the following way. Reference is made to the usual manner of carrying out the operation in a lithographic process. It is common practice first to make a set of color separation negatives. Screen positives are then prepared from these and the screen positives are then printed to form screen negatives. The latter are then printed on the prepared lithographic surface which usually consists of zinc or aluminum having a grained surface. Lithographic stones may also be used for the purpose but their use has largely been discontinued. It is customary, also, to perform whatever retouching is required on the screen positive. Heretofore it has been necessary to follow through this process to completion, that is, to the making of the final printing surface before a color proof could be obtained. By my invention I can obtain

such color proofs from the screen positive after it has been retouched and before making the screen negative and preparing the final printing surface. This, of course, saves a great deal of time. To accomplish this result I proceed in a manner analogous to that given above, as follows:

The method which I now propose may be used either with a screen positive or the screen negative made from it. The former method of using a screen positive is to be preferred, however.

I prepare a sensitive printing surface 10 composed of a white metal such as zinc or aluminum coated with asphaltum which has been sensitized with iodoform. This asphaltum is black and repellent to stain. This surface is exposed to light under the screen positive obtained in the usual lithographic process. The asphaltum coated metal is then developed with turpentine which washes off the asphaltum which has not been affected by light, presumably leaving as before an exceedingly thin layer. After briefly drying I then immerse this plate in a stain as given above which is repelled by the insoluble asphaltum. At this stage we have a design consisting of black asphaltum 11 and the background dye 12. This is shown in Figure 4. The asphaltum of the design is now removed by treatment with carbon tetrachloride. There now remains on the plate a positive dye image 12 with clear spaces 13 as shown in Fig. 5. To obtain a proof from this plate, I press into intimate contact with it a sheet of suitable paper which has been moistened with a solvent for the dye. The solvent extracts the dye from the plate and transfers it to the paper, giving a positive colored proof on the paper. To obtain a proof of the proper color, it is of course necessary to use a suitable dye for the stain but this can readily be accomplished as there is a very large assortment of satisfactory dyes. In this manner color proofs can be obtained from each of the color separation screen positives. If any portion of the proof appears unsatisfactory, it is only necessary to go back and modify the screen positive by retouching.

To obtain a color proof from the final screen negative it is necessary to add another step to the process thus mentioned. A sheet of white metal 20 is coated with bichromated shellac. After drying, this surface is exposed to light under the screen negative. It is then developed with denatured alcohol which removes the parts unaffected by light leaving a relief 21. Here as before there is presumably left an exceedingly thin layer of the shellac. After drying, this surface is brushed over with a solution of black asphalt in benzine. This is done by gently rubbing the surface with a tuft of cotton or a soft pad. The asphalt adheres to the plate

in the portions 22 where the shellac has been removed. This condition is represented in Figure 6. After the asphalt coating is dried, the shellac remaining is now removed with alcoholic ammonia. The surface is now flowed with the staining solution which is repelled by the asphalt, producing a dark asphalt image 22 in a dye background 23 as shown in Fig. 7. Finally, after again drying, the asphalt is removed, leaving a stain or dye positive 23 on the plate with colorless portions 24 therebetween. Since these portions have been obtained by different means, these layer portions may not be of equal thickness as shown (Figure 8). A proof can then be obtained from this plate in the same manner as before, that is, by pressing into contact with it a sheet of paper moistened with a solvent for the dye.

It is obvious that numerous methods of the practice and application of my invention are possible and I contemplate as included within my invention all such modifications and equivalents as fall within the scope of the appended claims.

What I claim is:

1. A process for making a copy of a printing image that comprises forming by photographic steps a layer having a relief image in which the relief is composed of portions which are repellent to stain and the other portions of which are receptive of stain, applying to the layer a stain which is contrastive in appearance with the repellent portions, and then transforming the stain repellent portions into non-repellent portions which are also contrastive with the stain.

2. A process for making a copy of a printing image that comprises forming by photographic steps a layer having a relief image in which the relief is composed of portions which are dark and repellent to stain and the other portions of which are receptive of stain, applying to the layer a stain which is adherent to said other portions, thereby producing an image of dark insolubilized portions in a stain background, and then transforming these last named portions into light colored portions.

3. A process for making a copy of a printing image that comprises exposing to light through the printing image a layer of material which is insolubilized by light, transforming this layer by a process which includes removal of the soluble portions into a relief image in which the relief is composed of insolubilized portions which are dark and repellent to stain and the other portions are receptive of stain, applying to the layer a stain which is adherent to said other portions, thereby producing an image of dark insolubilized portions in a stain background, and then transforming these last named portions into light colored portions.

4. A process for making a copy of a print-

ing image that comprises exposing to light through the printing image a layer of bi-chromated colloid, covering this layer with a greasy ink, then transforming this layer by removing the soluble portions into a relief image composed of insoluble colloid covered with ink, applying to the layer a stain which is adherent to the portions not covered by the ink, thereby producing an image of dark insoluble portions in a stain background, and then removing the ink.

5. A process for making a copy of a printing image which comprises exposing to light through the printing image a layer of bi-chromated albumen, covering this layer with a greasy ink, developing with water, applying to the layer a stain which is adherent to the portions not covered by ink, and then removing the ink.

6. A process for making a copy of a printing image that comprises forming by photographic steps a layer having a relief image in which the relief is composed of portions containing a substance which is repellent to stain and other portions receptive of stain, applying to the layer a permanent stain which is contrastive in appearance with the repellent portions, and then removing the repellent portions of said relief image, leaving the stain in the unprinted portions of said relief image.

7. A process for making a copy of a printing image that comprises exposing to light through a printing image a layer of material which is insolubilized by light, transforming this layer by a process which includes removal of the soluble portions into a relief image in which the relief is composed of insolubilized portions which are repellent to stain and other portions which are receptive of stain, applying to the layer a permanent stain which is adherent to said other portions, thereby producing an image of insolubilized portions in a stain background, and then transforming the insolubilized portions so that they are colorless and transparent.

8. A process for making a color print that comprises forming by photographic steps a relief image in an organic material in which the relief is the light affected portion, applying a stain dissolved in a medium which is not a solvent for said relief and therefore does not penetrate said relief, the stain affecting the low portion, removing the light affected portion of the relief image with a medium which is not a solvent for said stain, leaving the stain design and then transferring said stain design to a final support.

9. A process for making a color print that comprises forming by photographic steps a relief image in an organic material in which the relief is the light affected portion, applying a stain dissolved in a medium which is not a solvent for said relief and therefore does not penetrate said relief, the stain affecting the

low porton, removing the light affected portion of the relief image with a medium which is not a solvent for said stain leaving the stain design and then transferring said stain design to a final support by moistening the support with a solvent for said stain design.

Signed at Rochester, New York, this 6th day of March, 1930.

ALEXANDER MURRAY.

10

15

20

30

35

40

45

50

55

60

65